

## UNITED STATES PATENT OFFICE

2,370,130

## MANUFACTURE OF PROPELLANT POWDER

Leon W. Babcock, Wilmington, Del., assignor to  
Hercules Powder Company, Wilmington, Del.,  
a corporation of Delaware

No Drawing. Application April 11, 1941,  
Serial No. 388,083

12 Claims. (Cl. 52—22)

This invention relates to the production of colloided smokeless powder and more particularly to an improved method for pressing the smokeless powder colloid into the desired forms.

In manufacturing colloided smokeless powder of the single or double base type, it is necessary to force the material by means of presses into blocks and through forming dies. The pressure which is necessary to force the colloid into the desired form is usually supplied by means of a hydraulic ram under a pressure of 2,500 to 3,800 pounds per square inch. The smokeless powder during the pressing operations has been known to ignite and burn and in some instances has been known to explode. These combustions destroy the powder in practically all cases, often damage the press and expose operators to possible injury.

The object of this invention is to provide a method of pressing colloided smokeless powder which will prevent instances of ignition, fire or explosion.

A further object of this invention is to provide an improved method of operating the hydraulic presses used in the smokeless powder art.

A further object of this invention is to provide a safer method for forcing colloided smokeless powder through forming dies.

A still further object of this invention is to provide a method of pressing solvent-containing smokeless powder which will eliminate accidental ignition of the solvent vapors.

Other and further objects will be apparent hereinafter.

The objects of this invention have been accomplished by operating the hydraulic presses, in which the colloided smokeless powder is pressed in an atmosphere that is sufficiently inert to prevent the ignition and/or combustion of any vapors present, or of the smokeless powder within the press and to thus prevent the possibility of the vapors and/or powder from reaching a condition conducive to explosion. In particular, the powder is maintained in an atmosphere incapable of supporting combustion during the pressing operations and especially during the forcing of the powder through forming dies.

More specifically in accordance with this invention the possibility of ignition, combustion, or explosion of the material in the hydraulic presses

has been materially reduced or completely eliminated by regulating the composition of the gaseous medium within the press and/or within pockets in the powder. The gaseous medium within the press and within pockets or occluded in the powder is normally air and during the pressing operations will contain varying percentages of solvent vapors, such as for example, ether, acetone, alcohol or the like depending on conditions of temperature etc. Further, the air may contain varying percentages of any volatile compound which is contained within the smokeless powder. In accordance with this invention, the gaseous medium surrounding, in contact with and occluded by the powder is rendered inert, that is, incapable of supporting combustion by decreasing the percentage of oxygen therein. This decrease may be accomplished by sweeping out the press with inert gases such as nitrogen, carbon dioxide, helium, and the like or with inert gaseous mixtures, such as flue gas, exhaust gas, producer gas, and the like. Further, an oxygen deficiency may be accomplished by raising the concentration of the inert gas in the press such as, for example, by placing solid carbon dioxide in the press before the press is closed or by forcing inert gases into the press after it is closed. Decreasing the percentage of oxygen present produces a gaseous medium which will not support combustion and thereby prevents ignition, combustion or explosion within the press. The ignition or combustion which must be prevented is that of the solvent vapors as their ignition causes the ignition of the powder present, and once the powder is ignited, it will support its own combustion due to the available oxygen therein.

The colloided powder before blocking and pressing has been found to contain occluded gas and pockets of gas and in accordance with this invention this gas may be rendered inert and incapable of supporting combustion, since it is likewise compressed during operation and may ignite, burn, or explode during the pressing. Rendering non-explosive the gas which is in pockets or occluded within the powder may be accomplished by mixing the powder in an inert atmosphere or by treating the mixed powder with an inert atmosphere so that any occluded gas or pockets of gas formed in subsequent operations will be incapable of undergoing ignition.

The method in accordance with this invention may be employed in any step of smokeless powder manufacture where it is necessary to press the material such as by means of a hydraulic press. Thus, after the powder ingredients have been mixed especially with single base powders it is customary to force the lumpy material through what is known as a macaroni press. This press contains a perforated plate instead of specialized forming dies and the forcing of the smokeless powder through this plate insures proper mixing of the colloid. The method of preventing ignition, combustion or explosion by operating in an inert gaseous medium is applicable to this macaroni press. After the macaroni operation, the powder is blocked, that is, formed into a cylinder before it is put in the forming press. The blocking press may be operated under inert gaseous conditions. Further, with double base powder, the macaroni press may be used, but normally the double base powders after mixing are not put through the macaroni press but are immediately formed into blocks of powder suitable for insertion into final forming presses. The forming of the double base powder into blocks is also accomplished in a hydraulic press, and the method of this invention is applicable to this operation.

The actual pressing of the colloided powder into the desired size strands just prior to granulation is also accomplished by hydraulic presses. The presses may be of varying diameter but comparatively small presses, say four inches in diameter, are used for double base powder while large presses, say up to twenty inches in diameter, may be used for single base powders. The operation of these presses is made safer by controlling the gaseous medium therein so that an atmosphere incapable of supporting combustion is maintained.

It will be understood that the present invention may be used in any of the various hydraulic pressing operations necessary in the production of smokeless powder. Further, that the invention is applicable without special regard for the actual composition of the powder being pressed. The invention provides for means whereby the production of any of the numerous formulations of both single and double base powders may be accomplished in a safer manner.

In ignition, combustion, and/or explosion of the solvent vapors within the hydraulic presses is believed to be due in the main to the increase in the temperature of the gas phase occurring upon compression, but may be aggravated by friction or conditions which are undeterminable. The rate of compression, of course, controls the temperature rise but this rate is difficult if not impossible to control in operations due to variations in charges, weights, and vapor concentration. However, compression ratio must be considered and allowances made for most severe conditions. If the powder itself is ignited from any cause, the inert atmosphere will not snuff out the flame but ignition of the powder prior to ignition of the vapors is believed to be a rare occurrence.

To show that ignition may be reduced or eliminated by the method of this invention, Table I in which the effect on ignitability produced by the addition of two inert gases, nitrogen and carbon dioxide, to an alcohol-acetone vapor is presented below. The compression ratio in these experiments were closely controlled.

TABLE I  
*Suppression of compression ignition of acetone-alcohol vapor-air mixtures by inert gases*

| Type of vapor                | Combustible vapor concentration, volume, per cent | Inert gas, volume, per cent | Compression ratio * | Ignitability |
|------------------------------|---------------------------------------------------|-----------------------------|---------------------|--------------|
| Acetone-alcohol <sup>1</sup> | 8.0                                               | 0%                          | 16.8                | No ignition. |
|                              | 8.0                                               | 0%                          | 17.3                | Ignition.    |
|                              | 4.6                                               | 0%                          | 13.0                | No ignition. |
|                              | 4.6                                               | 0%                          | 13.3                | Ignition.    |
|                              | 2.2                                               | 0%                          | 12.1                | No ignition. |
|                              | 2.2                                               | 0%                          | 12.4                | Ignition.    |
|                              | 4.6                                               | 48% N <sub>2</sub>          | 22.9                | No ignition. |
|                              | 4.6                                               | do                          | 24.1                | Ignition.    |
|                              | 4.9                                               | 25.5% CO <sub>2</sub>       | 19.3                | No ignition. |
|                              | 4.9                                               | do                          | 21.0                | Ignition.    |
|                              | 4.6                                               | 48.5% CO <sub>2</sub>       | 54.1                | No ignition. |

<sup>1</sup> Liquid of the composition 62.5 anhydrous acetone and 37.5% ethyl alcohol (95 volume %) was used to saturate air at about 35° C. It was calculated from vapor pressure data that the vapor composition in equilibrium with this liquid contained about 30% acetone, 6% alcohol, and 1% water vapor (by volume). Thus the combustible vapor concentration was about 36%, and the above mixtures were obtained by diluting the concentrated vapor with the proper amounts of air or inert gas. Similar effects of inert gas were noted at other ratios of acetone to alcohol.

\* The underlined values show the minimum compression ratios at which it was possible to get ignition of the vapor mixtures. The maximum compression ratios at which non-ignition invariably was observed are also recorded. In case of the mixture containing 48.5% carbon dioxide, no ignition occurred at the maximum compression ratio convenient to apply in the apparatus used.

The apparatus used to study the compression ignition of solvent vapor-air mixtures given in Table I consists of a cylinder about two inches in diameter with a tight-fitting piston with a ten-inch stroke. The gas-vapor mixtures of a predetermined composition were introduced at normal temperatures into the cylinder at atmospheric pressure and the piston rapidly thrust into the cylinder to a predetermined compression ratio. The speed of the piston motion was such that adiabatic conditions prevailed. The super-heating of the gas-vapor mixtures brought about their explosion without any ignition device. By regulation of the compression ratios obtained, it was possible to determine a maximum compression ratio for which no ignition would occur and a minimum compression ratio for which ignition was certain to take place. These values are recorded in Table I above. By insertion of solvent wet smokeless powder in the bottom of the cylinder, it was found that adiabatic compression ignition of the solvent vapor-gas mixture was invariably followed by ignition and burning of the smokeless powder, whereas, when the conditions of the adiabatic compression heating of the gas phase were insufficient to cause its ignition, no ignition of the powder itself would occur.

The preferable method for controlling the composition of the gaseous medium in the hydraulic presses is by an injection valve entering through the ram or side of press, but many other methods are applicable for this control and such means as inserting solid carbon dioxide directly into the press, allowing a current of inert gas to continually sweep out the press either by entering the top or bottom openings, suitable valves within the operating mechanism, or by maintaining the entire press in an inert atmosphere are contemplated.

The advantages of the process of this invention is in the safety of operation, in the increased efficiency brought about by the lack of shutdown for repairs and in the increased production possible by increasing ram speeds. The elimination of

time and powder losses which occurred whenever ignition, combustion, or explosion occurred is also a great advantage.

It will be understood that the details and examples hereinbefore set forth are illustrative only and that the invention as broadly described and claimed is in no way limited thereby.

What I claim and desire to protect by Letters Patent is:

1. In the method of pressing colloided smokeless powder through dies by means of a hydraulic press, the step which comprises maintaining an inert atmosphere within the press during said pressing whereby ignition within said press is avoided.

2. In the manufacture of propellant powder of the single base type by mixing, pressing and granulating, the step which comprises maintaining an inert atmosphere in contact with the powder during the pressing operation whereby ignition of solvent vapors is prevented.

3. In the manufacture of propellant smokeless powders from admixtures comprising nitrocellulose and volatile solvents which includes mixing, pressing and granulating, the step of contacting said powder during said pressing with a gaseous medium containing sufficient nitrogen to render said medium incapable of supporting combustion whereby ignition of said solvent and said powder is prevented.

4. In the manufacture of propellant smokeless powders from admixtures comprising nitrocellulose and volatile solvents which includes mixing, pressing and granulating, the step of contacting said powder during said pressing with a gaseous medium containing sufficient carbon dioxide to render said medium incapable of supporting combustion whereby ignition of said solvent and said powder is prevented.

5. In the manufacture of propellant smokeless powders from admixtures comprising nitrocellulose and volatile solvents which includes mixing, pressing and granulating, the step of contacting said powder during said pressing with a gaseous medium containing sufficient exhaust gas to render said medium incapable of supporting combustion whereby ignition of said solvent and said powder is prevented.

6. In the manufacture of propellant powder from admixtures comprising nitrocellulose, liquid explosive nitric esters and volatile solvents, the

step of reducing the oxygen concentration of the gaseous medium in contact therewith to produce a gaseous medium characterized by non-ignitability, and pressing said powder in said reduced oxygen concentration through forming dies.

7. In the manufacture of propellant powder of the double base type by mixing, pressing and granulating, the step which comprises maintaining an inert atmosphere in contact with the powder during the pressing operation whereby ignition of solvent vapors is prevented.

8. The method of operating a smokeless powder extrusion press comprising loading the chamber of the press with a colloided admixture which

15 comprises nitrocellulose and volatile solvents, lowering the ram into the chamber of the press, introducing a current of inert gas into said chamber whereby the oxygen concentration of said chamber is reduced below the ignition point and then lowering the ram onto the admixture and extruding the admixture by application of pressure.

9. In the manufacture of propellant powder of the double base type by mixing, pressing, and granulating, the steps which comprise maintaining an inert atmosphere in contact with the powder during the mixing operation and during the pressing operation whereby ignition of solvent vapors is prevented.

10. In the manufacture of propellant powder of the single base type by mixing, pressing, and granulating, the steps which comprise maintaining an inert atmosphere in contact with the powder during the mixing operation and during the 35 pressing operation whereby ignition of solvent vapors is prevented.

11. In the manufacture of propellant powder of the double base type by mixing, pressing, and granulating, the steps which comprise maintaining a carbon dioxide atmosphere in contact with the powder during the mixing operation and during the pressing operation whereby ignition of solvent vapors is prevented.

12. In the manufacture of propellant powder of the single base type by mixing, pressing, and granulating, the steps which comprise maintaining a carbon dioxide atmosphere in contact with the powder during the mixing operation and during the 45 pressing operation whereby ignition of solvent vapors is prevented.

LEON W. BABCOCK.